

## UNITED STATES PATENT OFFICE

2,231,928

## METHOD OF TREATING CELLULOSIC MATERIAL

Christopher Luckhaupt, Jamaica, N. Y.

No Drawing. Application March 28, 1938,  
Serial No. 198,603

3 Claims. (Cl. 18—55)

This invention relates to a method of treating cellulosic material.

More particularly the invention relates to the treatment of cellulosic materials, such as pulp, sulfite, soda, kraft, wood or other cellulosic powder, pulp or fibrous matter. Examples of such materials include wood flour, newsprint, paper pulp, etc.

This application is a continuation in part of a part of my co-pending application Serial No. 75,929, filed April 23, 1936, entitled "Process of hardening cellulose matter and resulting products" now U. S. Patent No. 2,112,245, dated March 29, 1938, and a continuation in part of my copending application, Serial No. 113,463, filed November 30, 1936, entitled Method of treating porous materials and resulting products, now U. S. Patent No. 2,173,882, patented September 26, 1939.

An object of this invention is the treatment of cellulosic materials in the substantially raw or unprocessed stage to impart thereto enhanced hardness and enhanced correlated attributes, viz., increased tensile strength, increased flexural strength, increased compressional strength, oil- and water-proofness, fireproofness and the like.

An object of the invention is the production of processed material adapted to be utilized in the production of articles by molding processes, such as suction molding, pressure molding, and the like, usually with the aid of superheated steam.

An object of the invention is the production of cellulosic material resistant to weather deterioration, including resistance to the effects of the sun, and like exposure.

Another object of the invention is the production of cellulosic material embodying one or more of the above stated improved qualities and/or with variant coloring effect.

My invention comprises, in general, the treatment of porous matter of cellulosic character which is insoluble in warm terpin hydrate by subjecting the same in suitable relation with terpin hydrate, as by immersion in a suitable bath of the stated treatment material, or by subjecting such matter to a spray of such treatment material, or by subjecting such matter to the vapor arising from the hot treatment material. The aforesaid cellulosic materials as appears from my aforesaid U. S. Patent No. 2,173,882, patented September 26, 1939, are insoluble in the terpin hydrate treatment material at treatment temperature, to wit, at or above 115° C.

Further features and objects of the invention will be more fully understood from the following detail description.

Preferably my invention contemplates the addition to pulp, sulfite, soda, kraft and wood or other cellulose pulp or fibrous matter of similar material which is insoluble in the treatment material at or above 115° C., of terpin hydrate alone, in powdered form or terpin hydrate admixed with desirable fillers or fortifiers such as oleates, stearates, waxes, and gums, oils, both mineral and vegetable and which will have the effect of imparting desirable characteristics to the material being treated, or which will enhance characteristics already present in the material.

Where fortifiers are in liquid form, the same may be sprayed upon the material being treated or the material may be immersed in a volume of the fortifiers and afterwards removed therefrom, and excess fortifier expressed therefrom by pressure or gravity. The material being treated is ordinarily in finely divided form, such for example as so-called "wood flour," or finely divided pulp or ground-up pulp or in the case, for example, of old newsprint, the material is in the original form to be afterwards comminuted prior to subsequent molding processes.

The fortifiers, such as have been designated above, may be used simultaneously with or subsequent to the terpin hydrate, and in any event the fortifiers when employed are used in a quantity relative to the quantity of terpin hydrate in the ratio of substantially 2% to 50% of the quantity of terpin hydrate used. Further, a plurality of fortifiers may be used, and in such event, the amount of fortifiers used ranges from 2% to 50% of the quantity of terpin hydrate. The proportion of treatment material relative to the treated material is varied as desired, as is understood by those skilled in the art, depending upon the degree of impregnation by the treatment material of the treated material, the degree of the enhanced attributes of the resulting treated material varying with the proportion of the treatment material relative to the treated material, the treatment temperature above 115° C., and the duration of the treatment period.

The material treated according to my present invention remains in powdered or comminuted condition or may be powdered or comminuted after the process is complete.

Such treated material may be subjected to a molding process, such as suction molding or

- pressure molding with or without excess water, and usually with the aid of superheated steam and air. The material, after being subjected to the molding process, is then removed and allowed to dry, and upon drying attains the stage of substantial adhesion of the fibers, and the resulting article has all of the attributes of enhanced hardness, flexibility, immunity from action by water, oils, etc.
- 10 Color as desired may be imparted to the material and to the product resulting therefrom, by adding suitable coloring matter, such as animal, vegetable, mineral and other dyes, pigments, etc., simultaneously with the addition to the product of terpin hydrate.

Whereas I have described my invention by reference to specific forms thereof, it will be understood that many changes and modifications may be made without departing from the spirit 20 of the invention.

I claim:

1. The method of imparting enhanced hardness to cellulosic material, selected from pulp, sulfite, soda, kraft, and wood in comminuted form which is insoluble in terpin hydrate treatment material at treatment temperature of 25 115° C. and upward, which comprises admixing such comminuted material with terpin hydrate in powdered form, and then subjecting the cellulosic material to treatment temperature of 30

115° C. and upward and pressure in the presence of water.

2. The method of producing a molded product of cellulosic material selected from the group consisting of sulfite, soda and kraft pulp and 5 comminuted wood, said cellulosic material being insoluble in terpin hydrate at or above its melting point of approximately 115° C., which comprises treating said cellulosic material with terpin hydrate at or above 115° C. and subjecting 10 the resulting treated material to heat of the order of 115° C. and pressure in a suitable mold.

3. The method of producing a molded product of cellulosic material selected from the group consisting of sulfite, soda and kraft pulp and 15 comminuted wood, said cellulosic material being insoluble in terpin hydrate and a fortifier selected from the group consisting of oleates, stearates, waxes, and gums, oils, both mineral and vegetable, at or above the melting point of 20 the terpin hydrate of approximately 115 C., which comprises treating said cellulosic material with terpin hydrate admixed with such fortifier in the proportion of from 2% to 50% of 25 such fortifier to terpin hydrate at or above 115° C. and subjecting the resulting treated material to heat of the order of 115° C. and pressure in a suitable mold.

CHRISTOPHER LUCKHAUPT. 30